

## UNITED STATES PATENT OFFICE

MAX THIMANN, OF BERLIN-WILMERSDORF, GERMANY, ASSIGNOR TO THE FIRM DR. BEKK & KAULEN CHEMISCHE FABRIK G. M. B. H., OF BERLIN-LICHTERFELDE, GERMANY

## PROCESS FOR PHOTOCHEMICAL PRODUCTION OF ALUMINUM PRINTING FORMS

No Drawing. Application filed March 12, 1931, Serial No. 522,186, and in Germany March 17, 1930.

While it is easy in the photochemical production of zinc printing forms to remove the colloid coating from the exposed parts of the plate after having exposed, developed and etched the cleared parts of the plate before such removal is being made, for example by means of alkali, this removal of the hardened colloid coating makes difficulties when aluminum printing forms are used. 10 Alkali cannot here be used for the removal of the said coating, because it attacks the metal too strongly. By using acids, even strong acids, however, the removal of the coating does not as a rule occur, or only 15 with great difficulty, even not if at the same time some mechanical treatment is taking place.

It has now been found, that this drawback can be easily corrected, if the aluminum 20 plates or the like are first treated with acid-free solutions of salts from trivalent metals, before applying the sensitized colloid coating to the plate. Especially suitable for this purpose are the sulphates of aluminum, 25 chrome, iron and the like, and in first line the alums, such as potassic aluminum alum, iron ammonium alum, chrome potassium alum and so on.

By first treating the aluminum plate or 30 similar aluminum printing form with such a salt solution it is possible, easily to remove or wash off the parts of the coating hardened by exposure from the plate or the like, which after said treatment with the salt 35 solution has been covered with the sensitized colloid coating, exposed, developed and etched. This removing of the hardened coating can be easily and quickly done with suitable acids, especially phosphoric acid. 40 Thereby as a rule it is not dissolving of the hardened coating which takes place, but loosening of it from the metal plate or the like, so that the coating can be rinsed off the plate, either as a whole or in large pieces.

45 To attain the said effect it is, for example, sufficient to pour a diluted, say 1% solution of alum salt on to the clear metal plate, to leave it standing therewith for a short time, then to pour off the said solution and to 50 water the plate or the like and to coat it in

the usual way with a sensitized colloid-coating.

The further treatment, exposing, developing and, if desired, etching of the plate can be done in the usual way, wherein for etching the clear-laid parts of the aluminum plate or the like, preferably phosphoric acid, mixed with concentrated ferric-chloride can be used. By using the said mixture of phosphoric acid and ferric-chloride, for the preparation of which a ferric-chloride solution of at least 70% contents should be used, and which therefore has either the consistency of a paste or of a viscous fluidity, one attains, that the etching medium only acts on the clear-lying parts of the plate and does not go to the exposed parts of the plate through the hardened coating, which may be covered with a varnish or resin layer, if required.

To remove the coating from the etched 70 plate, a diluted phosphoric acid, e. g. a watery 10% phosphoric acid may expediently be used, whereby the loosening of the sensitized colloid coating from the plate previously treated with alum or the like, in 75 the way above stated, is easily attained.

If the plate, which has first been treated in the said way with salt solutions, then spread with the sensitized colloid coating, exposed and developed, is to be etched, the 80 parts of the plate to be protected from the action of the etching medium must be covered in known way with a suitable coating. In the above stated case, for an especially suitable cover-coating a mixture of tannable 85 organic substances, such as copying-glue, and tanning means, such as chrome alum are to be considered. The plate herein is treated for instance in that way, that a fresh mixture of about equal parts of copying-glue and a solution containing 5% chrome alum is brought on to the parts of the developed plate to be 90 protected. Here the mixture stiffens after some time owing to tanning setting in. The stiffening may be quickened by heating the 95 plate. The thus formed cover-coating protects the parts of the plate below it from the action of the etching means, for example from the above indicated mixture of phosphoric acid and iron chloride. The re- 100

- moval of the coatings on the plate after the etching by means of phosphoric acid can then be done forthwith, the protective coating formed from tannable substances and 5 tanning means being dissolved from the plate with the hardened gelatine coating in so far as the protective coating is arranged on the gelatine coating, but on the other hand also from those parts of the 10 plate where the protective coating is situated directly on the metal of the plate, it is directly dissolved without further ado by the action of the phosphoric acid.
- Having now particularly described and 15 ascertained the nature of my said invention, I declare that what I claim is:—
1. A process for the photochemical production of aluminum printing-forms, comprising treating the aluminum body with an acid-free solution of a salt of a tri-valent metal, coating a sensitized-colloid coating onto the plate, exposing, developing, and etching the plate, and then removing the 20 hardened colloid-coating.
  2. A process according to claim 1 in which the salt for treating the aluminum body, prior to applying the sensitized colloid-coating, consists of an acid-free solution of a sulphate of a tri-valent metal. 25
  3. A process according to claim 1, in which the salt for treating the aluminum body, before applying the sensitized colloid-coating, consists of an acid-free solution of an alum. 30
  4. A process for the photochemical production of aluminum printing-forms, comprising treating the aluminum body with an acid-free solution of a salt of a tri-valent metal, coating a sensitized-colloid coating onto the plate, exposing, developing, and etching the plate, and then removing the 35 hardened colloid-coating by means of a dilute acid. 40
  5. A process according to claim 4, in which the hardened colloid-coating remover is a water solution of phosphoric acid. 45
  6. A process for the photochemical production of aluminum printing-forms, comprising treating the aluminum body with an acid-free solution of a salt of a tri-valent metal, applying a sensitized colloid-coating thereover, exposing and developing the 50 plate, etching the clear-lying parts of the plate with phosphoric acid, and removing the hardened colloid-coating from the metal with dilute phosphoric acid. 55
  7. A process for the photochemical production of aluminum printing-forms, comprising treating the aluminum body with an acid-free solution of a salt of a tri-valent metal, applying a sensitized colloid-coating thereover, exposing and developing the 60 plate, etching the clear-lying parts of the plate by means of a mixture of phosphoric 65

acid and highly concentrated ferric-chloride, and removing the hardened colloid-coating from the metal by dilute phosphoric acid.

8. A process for the photochemical production of aluminum printing-forms, comprising treating the aluminum body with an acid-free solution of a salt of a tri-valent metal, applying a sensitized colloid-coating thereto, exposing and developing the plate, 70 covering those of the developed parts of the plate which it is desired to protect against etching with a protective coating, said coating consisting of a tannable, organic substance and a tanning-instrumentality, etching the plate, and removing the hardened colloid-coating together with the said protective coating by means of dilute phosphoric acid. 75

In testimony whereof I have hereunto set 80 my hand.

MAX THIMANN.

90

95

100

105

110

115

120

125

130